

1

2,946,782

## PROCESS FOR THE MANUFACTURE OF VISCOSE RAYON STAPLE

Shozo Tachikawa, Higashiyama-ku, Kyoto, Japan, by mutual agreement of all the heirs of said Shozo Tachikawa, deceased, to Tatsuji Tachikawa, heir

No Drawing. Filed Apr. 5, 1957, Ser. No. 650,818

4 Claims. (Cl. 260—217)

This invention relates to a process for producing rayon staple or filament having a high degree of polymerization (D.P.) from alkali cellulose.

Various expedients are known to the rayon art for preventing decomposition of the alkali cellulose and the xanthate radicals in the several stages of manufacture. The problem is particularly acute where the starting cellulosic material has a high D.P. According to the invention the alkali cellulose is xanthated with carbon disulphide and a surface active agent in the presence of a mono amine. The use of mono amine has hitherto been confined to the spinning or coagulating and regenerative steps in the viscose to rayon stage of the process where it is employed as an additive to the viscose for controlling the primary gel swelling of the extruded filament and for increasing the tenacity of the rayon fibers or where it has been used in the production of viscose itself its use has been restricted to the stage previous to xanthation such as in the alkali cellulose steeping stage. The mono amine is adapted to react with the zinc sulfate in the spinning bath to produce these desirable properties in the final product. While in the process of this invention mono amine exists in the spinning bath to impede the decomposition of the xanthate radicals and to facilitate spinning in a weak acid bath, the introduction of this ammonia base salt is actually made in the previous xanthation stage. It has been found that the mono amine causes the carbon disulphide to mix easily with the surface active agent as it is soluble in each liquid. Consequently, the penetration of the carbon disulphide into the cellulose occurs at an accelerated rate of xanthation. Due to the presence of the mono amine in the cellulose xanthate, the decomposition of the xanthate radicals is restricted and there is produced a xanthate having a high  $\gamma$  (gamma value) i.e. number of xanthate radicals per 100 glucose units of one cellulose molecule. Additionally, the xanthate radicals are more uniformly distributed in the viscose.

The advantages of employing the particular xanthating step of this invention are principally fivefold. Firstly, the process may employ cellulose material of very high D.P., for example 1000 to 1200 without sacrificing viscosity, which for the viscose is usually more than 200 seconds by the ball drop test; secondly, the viscose as produced by applicant's process is easily spun in a low acid bath at a rate of 30 to 70% higher than for conventional processes. The acid concentration of the bath may be below 20 grams per liter, which is principally due to the high viscosity of the easily spun high D.P. viscose; thirdly, the rate of xanthation is accelerated and the distribution of the xanthate radicals in the xanthate is uniformly improved; fourthly, a regenerating or secondary bath may be employed in addition to the initial coagulating bath in the spinning stage and tension may be applied to the thread in the secondary bath without imposing on the regenerating material any undue strain. When the material has decomposed unduly in any stage

2

of the process, this second bath may not be employed without sacrificing some of the desirable properties of the finished product. Because the decomposition of the xanthate radicals is controlled by the presence of the mono amine, the regenerating bath may be satisfactorily employed; and, fifthly, the properties of the rayon staple or filament produced by the instant process are improved over those achieved by other processes. The properties of the spun thread are easily controlled while it is passing through the secondary bath as by properly correlating the stretching ratio to the regenerating conditions on a stepped or conical godet as shown in my Patent No. 2,732,279. Both the axial properties, such as dry and wet tensile strengths, and the lateral properties, such as knot tenacity and flex life, of the finished rayon are improved as a result of the invented process.

It is to be noted that no component other than sulfuric acid is required for the spinning bath. It is unavoidable, however, that sodium sulfate will accumulate in the spinning bath. Yet in practice the sodium sulfate was found not to exceed 60 grams per liter. Mono amines suitable for the purpose of the present invention have generally the formula  $R_1R_2R_3N$ , in which at least one  $R$  is an alkyl radical and the remainder H atoms. It was found that a practical range of amines is 0.5 to 4.0% based upon the weight of the starting pulp; it is not necessary to use more than 4.0% of the agent to produce effective results.

The relation between the D.P. of the starting material and the spinning conditions is shown in Table 1 which compares the instant process with a former process which did not employ an amino salt in the xanthating solution.

TABLE 1

|                                         | Present Process |           | Former Process |
|-----------------------------------------|-----------------|-----------|----------------|
|                                         | A               | B         |                |
| D.P. of starting material.....          | 700-900         | 800-1,200 | 700-900        |
| Acid con. of spinning bath (g./l.)..... | 5-20            | 3-10      | 8-30           |
| Spinning velocity (m./min.).....        | 25              | 20        | 15             |
| Application of secondary bath.....      | possible        | possible  | unsuitable     |

The properties of the product prepared by the process of the present invention are shown in Table 2 in comparison with those of the former process.

TABLE 2

|                               | Present Process |      | Former Process |
|-------------------------------|-----------------|------|----------------|
|                               | A               | B    |                |
| Denier (d.).....              | 1.15            | 1.14 | 1.53           |
| Dry tenacity (g./d.).....     | 4.27            | 5.09 | 3.33           |
| Wet tenacity (g./d.).....     | 3.08            | 3.61 | 2.51           |
| Dry elongation (percent)..... | 12.1            | 12.9 | 9.8            |
| Flex life (cycle).....        | 600             | 900  | 300            |
| Knot tenacity (g./d.).....    | 2.04            | 2.45 | 1.87           |
| D.P. ....                     | 500             | 700  | 500            |

By the application of this process, the product was improved by 60% in dry tenacity, 40% in wet tenacity, 30% in dry elongation, 200% in flex life and 30% in knot tenacity respectively, in comparison with those of the former process.

As related fully hitherto, conspicuous improvements were achieved by the present invention for the various properties of high D.P. viscose rayon staple or filament.

## Example 1

Wood pulp having a D.P. of 750 is steeped in 18% caustic soda solution at 20° C. for 2 hours, squeezed to

2.65 times the initial weight of the pulp, shredded at 15° C. to 25° C. for 2.5 hours with a mixture of carbon disulphide of 53%, triethylamine of 3.5% and Turkish red oil of 2% based on the initial weight of the pulp respectively. The cellulose xanthate thus obtained is dissolved in a diluted caustic soda solution to obtain a viscose having the viscosity of 350 sec. with the cellulose concentration of 5% and total alkali concentration of 3%. After filtering and deaeration, the viscose is extruded into the spinning bath containing sulfuric acid of 12 g./l. and thereafter the gel thread is stretched step by step on a four-stepped godet (the ratio of consecutive steps is 1:2, 2:5, 5:3) immersed in the spinning bath. The thread is successively treated in a regenerating bath containing sulfuric acid of 15 grams per liter at 85° C. under stretching ratio of 15%. The final spinning velocity is 20 meters per minute.

The properties of the rayon staple or filament prepared by the process described herein are summarized on the second column of Table 2.

*Example 2*

Wood pulp having a D.P. of 1100 is steeped in 18.5% caustic soda solution at 20° C. for 2 hours, squeezed 2.7 times the initial weight of the pulp, and shredded at 25° C. for 1.5 hours and the alkali cellulose thus obtained is successively xanthated at 18° C. to 28° C. for 2.5 hours with a mixture of carbon disulphide of 55%, triethylamine of 1% and Turkish red oil of 2% based on the initial weight of the pulp respectively. The cellulose xanthate thus obtained is dissolved in a diluted caustic soda solution to obtain a viscose having the viscosity of 550 sec. with the cellulose concentration of 5% and total alkali concentration of 3.5%. After filtering and deaeration, the viscose is extruded into the spinning bath containing sulfuric acid of 4.8 grams per liter and thereafter the gel thread is stretched step by step on a five-stepped godet (the ratio of consecutive steps is 1:2, 2:5, 5:3, 3:2) immersed in the spinning bath. The thread is successively treated in a regenerating bath containing sulfuric acid of 40

6 grams per liter at room temperature without tension.

The properties of the rayon staple or filament prepared by the process described herein are summarized in the third column of Table 2.

5 It is to be understood that various modifications may be made in the disclosed process without departing from the scope of invention as defined in the appended claims.

What is claimed is:

10 1. In the production of viscose, a process for xanthating alkali cellulose comprising the step of introducing shredded alkali cellulose into a xanthating medium containing carbon disulphide, Turkey red oil as a surface active agent and a monoamine having a formula  $R_1R_2R_3N$  in which at least one R is an alkyl radical and the remaining R's are H atoms.

15 2. A process for xanthating shredded alkali cellulose as claimed in claim 1 in which the range of the monoamine in the xanthating solution is from 0.5% to 4.0% based on the weight of the starting pulp.

20 3. A process for xanthating shredded alkali cellulose as claimed in claim 2 in which the monoamine is triethylamine.

25 4. In the production of viscose, a process for xanthating alkali cellulose comprising the step of introducing shredded alkali cellulose into a xanthating medium containing carbon disulphide, a surface active agent and a monoamine having a formula  $R_1R_2R_3N$  in which at least one R is an alkyl radical and the remaining R's are H atoms.

References Cited in the file of this patent

UNITED STATES PATENTS

|           |           |               |
|-----------|-----------|---------------|
| 2,432,127 | Schlosser | Dec. 9, 1947  |
| 2,535,044 | Cox       | Dec. 26, 1950 |
| 2,592,355 | Tachikawa | Apr. 8, 1952  |
| 2,647,114 | Torke     | July 28, 1953 |
| 2,663,704 | Yehling   | Dec. 22, 1953 |
| 2,732,279 | Tachikawa | Jan. 24, 1956 |
| 2,855,321 | Bachlott  | Oct. 7, 1958  |